

## UNITED STATES PATENT OFFICE

1,939,170

BASE FOR USE IN THE MANUFACTURE OF  
HEAVY OILS AND GREASES

Alexander Horwitz, New York, N. Y.

No Drawing. Application April 2, 1931  
Serial No. 527,360

4 Claims. (Cl. 87-9)

This invention relates to a base for use in the manufacture of heavy oils or greases; and the object of the invention is to provide a base of the class specified, which will produce a product 5 of the class referred to having highly viscous and stringy characteristics; a further object being to provide a base of the class specified, which may be readily combined or compounded with suitable mineral oils in the production of a heavy 10 oil or grease and wherein the base may be distributed in the form of a powdered or granular product or in the form of a jelly-like product as desired; a still further object being to provide a base which will in compounding with a mineral oil, produce a product having a constant or relatively permanent viscosity; and with these 15 and other objects in view, the invention consists in a base of the class and for the purpose specified, compounded in the manner hereinafter more 20 fully described and claimed.

My invention consists in combining or compounding a metallic, water insoluble soap with glycerine, preferably chemically pure. If desired, I may add in the compounding of the 25 base, an oil having relatively high lubricating value, such as sperm oil or castor oil, or a compound of same, the latter being mixed with the glycerine in compounding with the metallic soap.

It will be understood that the amount of glycerine employed as well as added oil, if employed, will be varied to suit the particular grade and characteristics of the mineral oil with which the base is compounded in forming the heavy lubricating oil or grease, and also depending upon the 35 desired characteristics of the resulting product, it being understood that the lubricating oil or grease made from the base may be produced in different grades or qualities.

In the desire to produce products of this class 40 having high lubricating value as well as viscosity and the desired stringy characteristics, when the base is combined with mineral oils of a high viscosity and lubricating value, a relatively small amount of the base will be necessary—and with 45 lower viscosity oils, a higher percentage of the base, or the addition of sperm oil or castor oil will be necessary when extra lubrication is desirable. As one example of producing my improved base, I add or compound approximately 50 5% of glycerine, preferably chemically pure, to 95% of a metallic soap, such as aluminum stearate.

In producing the base, 5% of glycerine is first stirred thoroughly with about 10% of the aluminum stearate, and after thoroughly combined,

the remainder of the aluminum stearate is gradually added, while the mass is constantly stirred, the resulting product resembling a powdered or granular base which may be packed and shipped to oil or grease makers, and combined or compounded with a mineral oil as later set forth.

Instead of proceeding as above, I may first combine the glycerine with about 20% of water to produce a larger liquid volume, facilitating the initial introduction of a greater amount of the aluminum stearate, for example, about 50%, and the quicker mixing or compounding of the stearate with the glycerine. After being thoroughly compounded, the resultant mass may be subjected to heat at about 180° to 190° Fahrenheit, 70 the mass being stirred or agitated to prevent melting of the aluminum stearate, and this operation continues until the water initially introduced in compounding, is evaporated.

When it is desired to add lubricating value to 75 the base to increase the lubricating value of the resulting oil or grease made from the base, I preferably incorporate in the base, an oil or oils of high lubricating value, such for example as sperm oil or castor oil. The percentage of such 80 oil introduced will depend largely upon the results desired in the finished product made from the base. As one example, I compound with 5% glycerine, 12% sperm oil and 8% castor oil, and to this compound 75% of metallic soap such as 85 aluminum stearate introduced while thoroughly stirring the product, and the resulting base produced from this compounding will be of a granular or powdered character having slight greasy or oily characteristics.

In connection with the production of the bases above referred to, it will be understood that if desired, the base may be produced in the form of a jelly-like mass by incorporating with the base in its compounding, a sufficient amount of a mineral oil to produce the jelly-like product. The 95 advantage of producing the jelly-like product is that it simplifies the production of the resulting oil or grease by the oil or grease maker, it being understood that a lesser amount of the mineral oil is required in the production of the desired product, and such mineral oil may be more readily compounded with the jelly base by reason of the fact that the melting point of the jelly-like base is lower than the powdered or granular 100 base.

In the production of a predetermined amount of heavy oil or grease from the powdered base, approximately 3% or more of the base is incorporated with the computed amount of oil or 110

grease to be produced in the following manner. The desired percentage of base is first compounded with about one third of the mineral oil, subjecting the same to heat at about 220° Fahrenheit, thoroughly and continuously stirring the mass in this operation until the base is dissolved in the oil and the resulting product is clear, after which the balance of the two thirds of the oil is slowly added, while continuing to stir the mass until all of the oil has been thoroughly incorporated and the resulting product is clear. Depending upon the amount of mineral oil and the percentage of the base incorporated therein, the resulting product will resemble a very heavy oil or a grease, both of which products will be of a stringy consistency.

A product produced according to my invention will possess substantially constant viscosity and will be found to be of exceeding value as a lubricant for apparatus or machinery of various kinds and classes, wherein the rotating or reciprocating parts subjected to the lubricant will draw or carry the lubricant with the rotating or reciprocating element, by virtue of the viscous or stringy characteristics of the oil, thus insuring better lubrication.

In referring to the stringy characteristics of my product, by this I mean, that in dipping into a mass of the heavy oil or grease and attempting to remove a portion of the mass, a heavy string-like body will join the initial mass with that portion thereof which is removed, and this body, while still intact with both the mass and the removed portion of the mass may be engaged between two fingers of the hand and stretched laterally. It will be understood at this time, that the degree of stringy characteristics to the resulting, heavy oil or grease may be varied to suit specific requirements.

40

It will be understood that my invention is not limited to the various proportions or characteristics of the ingredients herein set forth, and from experience, I have found that as low as 1% of glycerine may be incorporated with a metallic soap, such as aluminum stearate, to produce a base which when compounded with a mineral oil, will produce a viscous stringy product. It will also be apparent that I may use as low as one half of 1% of the base in compounding with mineral oil, to increase the viscosity of such oil. Various other changes in and modifications of the invention herein set forth may be made within the scope of the appended claims, without departing from the spirit of my invention or sacrificing its advantages.

Having fully described my invention, what I claim as new and desire to secure by Letters Patent, is:

1. A base of the class described produced in compounding approximately 95% of aluminum stearate with 5% of glycerine.

2. A base of the class described produced in compounding approximately 75% of aluminum stearate with 5% of glycerine including 12% 100 sperm oil and 8% castor oil.

3. A base for producing a lubricant having viscous, stringy characteristics comprising aluminum stearate with which is compounded glycerine in substantially the proportions of 75% of 105 aluminum stearate and 5% of glycerine.

4. A grease base of the class described comprising aluminum stearate with which is compounded glycerine substantially in the proportions 95% of aluminum stearate and 5% of glycerine and 110 substantially five per centum of said base being compounded with a mineral oil in the production of a highly viscous and stringy lubricant.

ALEXANDER HORWITZ.

115

45

120

50

125

55

130

60

135

65

140

70

145

75

150